

## UNITED STATES PATENT OFFICE

CAMILLE DREYFUS, OF NEW YORK, N. Y., AND WILLIAM WHITEHEAD, OF CUMBERLAND, MARYLAND, ASSIGNEES TO CELANESE CORPORATION OF AMERICA, A CORPORATION OF DELAWARE

## SAPONIFICATION OF CELLULOSE ESTERS

No Drawing. Application filed June 20, 1928. Serial No. 287,035.

This invention relates to the treatment of products made from or containing inorganic esters of cellulose and is directed particularly to an improved method of saponifying such inorganic esters of cellulose.

5 An object of this invention is to provide a process for the saponification of inorganic cellulose ester materials whereby the valuable properties of the material will be enhanced.

10 Another object of this invention is to saponify the inorganic cellulose esters under such conditions that a material of greatly increased strength is obtained.

15 Still another object of our invention is to render yarns, films, etc., containing inorganic esters of cellulose capable of absorbing atmospheric humidity and becoming more suitable for working in textile operations.

20 Another object of this invention is to treat nitrocellulose in such a manner that its inflammability is greatly reduced but its valuable properties are retained. Other objects and advantages of this invention will appear from the following detailed description.

25 All of the saponification processes suggested to date have utilized an aqueous solution of an alkali or other material which would yield free hydroxyl ions in solution.

30 This saponification treatment, however, was objectionable since in addition to the great loss in weight, it resulted in the cellulose esters losing most of their distinctive and desirable properties such as strength, elasticity, hand appearance, etc. Also the saponification yielded a regenerated cellulose which material is rather weak in tensile strength. Moreover, with the old process it was difficult to control the saponification so as to yield a product which was uniform in appearance and evenly saponified.

35 It was also known that nitrocellulose possessed some properties which were very much desired in materials used for textile purposes. 40 However, the use of this particular ester of cellulose in the textile field has been practically nil because of its high inflammability and because the denitrating processes heretofore employed have not only reduced its inflammability but at the same time adversely

affected the other valuable properties of the nitrocellulose. Our invention has overcome this difficulty since it results in the saponification of the nitrocellulose without deleteriously affecting the properties which render it useful for textile purposes.

45 We have now found that if the saponification of the cellulose esters is effected by introducing the ester or ester materials into an atmosphere of or containing ammonia gas and water vapor, the product remaining differs in its properties from that obtained by known saponification methods. The nature of the saponification reaction is apparently changed and a greater degree of control of the reaction is permissible. By proper control of this method of saponification, it is possible to obtain a cellulose ester which will not take cotton dyes. It is possible by this 55 method to effect a virtually complete saponification of the cellulose nitrate in a comparatively short time. The cellulose which remains after such complete saponification possesses desirable qualities which are not 60 found in regenerated cellulose.

65 The cellulose nitrate materials treated in accordance with this process possess another marked advantage, not only over materials saponified by other known methods but also over the cellulose ester materials in their 70 original state. This is their remarkable increase of strength as compared with saponified cellulose or cellulose esters saponified by the old methods. In several instances the 75 increases in the dry tensile strength of the yarn treated in accordance with this invention has been higher than 30%, even though the yarn has been saponified over 95%.

80 Cellulose nitrate material due to its high inflammability cannot, of course, be ironed and this has been one of the factors precluding its use for textile purposes. We find that nitrocellulose material which has been 85 virtually completely saponified in accordance with this invention can be subjected to such temperatures as are usually utilized in ironing without any deleterious effects upon the material. This desirable result is effected by subjecting the nitrocellulose material to 90 the action of an atmosphere of, or containing, 95

100

a base and water vapor at comparatively low temperatures. Enough of the saponifying medium should be present to effect the desired amount of saponification.

5 The material to be treated can be in any desired form such as yarn or thread in hanks or on bobbins or pirns, in the form of knitted or woven fabric, garments or in the form of films, bristles, etc. The desired gaseous 10 atmosphere can be obtained in any suitable manner for instance, by suspending the cellulose ester material in a large aspirator connected with a container having therein a 28% solution of ammonia or other volatile base. 15 Without desiring to be limited to such specific concentrations or particular reagents it can be stated that very good results were obtained by first extracting the cellulose ester material to remove any lubricants which 20 might be present, drying the material at 100° C. and then subjecting the same to the action of an atmosphere saturated with ammonia and water vapor at temperatures of 25° C. to 30° C. The cellulose nitrate material was suspended in a large aspirator connected with a flask containing an ammonia solution. The time during which the reaction is allowed to proceed will vary depending upon the extent of saponification desired. 30 Thus at the end of 4 hours an approximate saponification of 2.5% was found; at the end of 6 hours 10.1%; at the end of 8 hours 63.1%; at the end of 16 hours 99.8%. The time can be shortened by utilizing a slightly 35 higher temperature for the reaction atmosphere but the lower temperatures are preferable since they result in a more uniform saponification.

The materials which may be used to effect 40 the saponification can be ammonium hydroxide, methyl amine, dimethyl amine or any other volatile base which will yield hydroxyl ions under the conditions of operation. The base selected, however, should be

45 compatible with water vapor since the latter must be present in the reaction atmosphere. As previously stated, good results were obtained utilizing an aqueous solution of ammonia of approximately 28% strength.

50 This process is applicable not only to yarns, threads, films, etc., made of or containing cellulose nitrate but also can be applied to such cellulose ester materials when they are admixed or formed with other fibres, whether 55 the latter are animal, vegetable or artificial in nature. Thus a fabric containing cellulose nitrate in admixture with cotton, wool, silk, linen, reconstituted cellulose (rayon) can be effectively treated in accordance with 60 this invention.

The fact that the cellulose remaining after 65 complete saponification according to our invention is different from normally regenerated cellulose is further evidenced by the increase in strength or tenacity noted in the

saponified yarn. This indicates that while there has been a loss of nitro radicals in the cellulose molecules there has been only a slight loss of bonds between the cellulose molecules themselves which constitute the 70 yarn, a result quite opposite to that resulting from the normal saponification.

As an example of a method of carrying out our invention, we give the following:

#### Example

Skeins of cellulose nitrate were extracted to remove lubricants, dried at 100° C. and weighed. These skeins were then conditioned in normal atmosphere and then suspended in a large aspirator connected with a flask containing an aqueous solution of ammonia of 28% strength. The aspirator was sealed and a very thin layer of ammonia solution maintained on its base. About every hour during the first eight hours of reaction, the skeins were shaken out and turned. The temperature in the aspirator was maintained at 27° C. to 29° C. The yarn employed was 80 150 denier and contained 26 filaments and 85 had an approximate nitro value of 51.7%.

At the end of 2 hours, cellulose nitrate treated as above was found to be saponified 1.15%; at the end of 5 hours, 5.1%; at the end of 7 hours, 31.7%; at the end of 8 hours, 63.1%; at the end of 10 hours, 97.2%; at the end of 16 hours, 99.8%. Even when saponified as much as 63%, the material was resistant to cotton dyes. Cellulose nitrate materials saponified in accordance with this invention were found to possess a pronounced 90 resistance to delustering on boiling when the percentage of saponification exceeded 90%.

Another distinctive property of the saponified material is the percentage regain of moisture. This is a very valuable property for not only does it offset the loss in weight due to saponification but it also renders the material more pliable. This is desirable for yarns of 100 cellulose ester material since it renders them more suitable for use in the various textile operations. This is especially true of nitro esters of cellulose.

The following table shows the percentage 115 regain of moisture of cellulose nitrate after saponification.

| Per cent saponification | Per cent regain |
|-------------------------|-----------------|
| Blank—none              | 2.82            |
| .58                     | 2.94            |
| 1.15                    | 3.20            |
| 1.71                    | 3.51            |
| 2.5                     | 4.03            |
| 5.1                     | 4.75            |
| 10.1                    | 5.89            |
| 31.7                    | 7.62            |
| 63.12                   | 8.54            |
| 97.2                    | 9.45            |

The resistance of the cellulose nitrate material to heat is very largely increased.

Whereas the material in its original condition could not safely be subjected to ironing, even at comparatively low temperatures, the saponified material can be safely ironed at 5 temperatures as high as 260° C. without any danger of inflammability and without any deleterious effect on the cellulose material.

While the specific description has dealt largely with cellulose nitrate, the invention 10 is not to be considered as limited thereto but is applicable to all inorganic esters of cellulose and the term "inorganic cellulose esters" as used in the claims is to be so interpreted. The term "% of saponification" as used in the 15 description and claims is calculated on the loss in dry weight and is quoted as % of nitro groups lost, assuming an original nitro value of 51.7%.

Having described our invention what we 20 claim and desire to secure by Letters Patent is:

1. Process of saponifying inorganic esters of cellulose which comprises subjecting materials containing the same to the action of a 25 saponifying agent in vapor form under such conditions as to at least partially saponify the cellulose esters and in the presence of moisture.

2. Process of saponifying materials containing inorganic esters of cellulose which comprises treating the same with a vaporous saponifying agent in the presence of moisture.

3. Process of saponifying materials containing cellulose nitrate which comprises treating the same with a vaporous saponifying agent in the presence of moisture.

4. Process of saponifying materials containing inorganic esters of cellulose which 40 comprises subjecting the same to the action of an atmosphere containing ammonia and water vapor, the amount of ammonia present being sufficient at least partially to saponify the inorganic esters of cellulose.

5. Process of saponifying materials containing cellulose nitrate which comprises subjecting the same to the action of an atmosphere containing ammonia and water vapor, the amount of ammonia present being sufficient at least partially to saponify the cellulose nitrate.

6. Process of saponifying materials containing cellulose nitrate which comprises subjecting the same to the action of an atmosphere resulting from the vaporization of a 55 28% aqueous solution of ammonia.

7. Process of saponifying materials containing cellulose nitrate which comprises subjecting the same, at temperatures not above 60 30° C., to the action of an atmosphere resulting from the vaporization of a 28% aqueous solution of ammonia.

8. Process of increasing the tensile strength of cellulose nitrate materials which 65 comprises saponifying the cellulose nitrate

material with a saponifying agent in vapor form under such conditions as to at least partially saponify the cellulose nitrate and in the presence of moisture.

9. Process of increasing the tensile 70 strength of materials containing cellulose nitrate which comprises saponifying the cellulose nitrate material in an atmosphere containing ammonia and moisture in vapor form.

10. Method of treating textile material containing filaments of inorganic esters of cellulose comprising at least partially saponifying the inorganic esters of cellulose with a saponifying agent in vapor form in the presence of 80 moisture.

11. Method of treating textile material containing filaments of cellulose nitrate comprising at least partially saponifying the cellulose nitrate with a saponifying agent in 85 vapor form in the presence of moisture.

In testimony whereof, we have hereunto subscribed our names.

CAMILLE DREYFUS.

WILLIAM WHITEHEAD. 90

95

100

105

110

115

120

125

130